# EUROPEAN PATENT SPECIFICATION

(11) **EP 0 060 948 B1**
(45) Date of publication and mention of the grant of the patent: **20.03.1985**
(21) Application number: 81301272.1
(22) Date of filing: 25.03.1981
(51) Int. Cl.: D21H 5/26, D04H 1/72

(54) **Methods for forming nonwoven fibrous webs**
Verfahren zur Bildung nichtgewebter faseriger Vliese
Méthodes de formation de nappes fibreuses non-tissées

(43) Date of publication of application: 29.09.1982
(73) Proprietor: James River-Norwalk, Inc., Norwalk Connecticut 06856 (US)
(72) Inventor: Widnall, Sheila E., Lexington Massachusetts 02173 (US)
(74) Representative: Slight, Geoffrey Charles

## Description

This invention relates to methods for forming nonwoven fibrous webs, wherein a layer of fibers is deposited from a gaseous suspension of fibers onto a moving foraminous forming surface. More specifically, this invention provides improvements in methods of achieving high speed production of nonwoven fibrous webs.

In the production of nonwoven webs, the prior art has generally disclosed systems which form an air suspension of fibers and direct the suspended fibers toward a moving foraminous forming surface upon which the fibers from the suspension are condensed-to form the nonwoven web. Various apparatuses exist for generating the air suspension of fibers. The fibers, for example, can be produced by a lickerin, a hammermill, or by other apparatus known in the art. The fibers can be dispersed in a gaseous medium by a variety of methods, and conveyed to a forming surface in an air stream operating generally as a pressure flow system, a vacuum system or a closed loop system. We have found that critical process limitations exist in the production of such air laid nonwoven webs, and that in a given system the uniformity of the formed web tends to decrease as the speed of the forming surface increases. It has been found that particularly at commercial speeds above about 550 feet per minute (2.79 meters per second), fiber lay-down on the moving forming surface tends to become uneven in the machine direction (i.e. the direction of travel of the forming surface). Thus the deposited webs exhibit an upper surface having an undulating, wave-like or ripple effect extending transverse to the machine direction, so that the webs exhibit corresponding variations in thickness and in weight. This rippling effect becomes more pronounced as the speed of the forming surface increases, with the spacing between the thicker portions of the web becoming greater and with the web becoming more varied along its surface as to basis weight. This rippling effect worsens with increased speed and eventually renders webs commercially unacceptable at some higher speed. This invention has sought to alleviate significantly the detrimental ripple effect. We have determined that there exists a critical relationship between the velocity of the fibers relative to the velocity of the moving forming surface as the fibers are being deposited onto the forming surface. We have found that the detrimental ripple effect can be controlled by controlling the ratio of the tangential velocity of the fibers relative to the moving forming surface, as compared to the velocity of the fibers normal to the moving surface.

Prior art concerned with obtaining higher production speeds in the production of air laid webs includes U.S. Patent No. 4,004,323 wherein it is taught that speeds in excess of 200 feet per minute (1.01 m/sec) and even in excess of 400 feet per minute (2.03 m/sec) can be achieved by inclining a duct, which carries a stream of fibers, at an angle to a forming surface. The patent teaches a range of angles of incidence of the duct relative to the forming surface of from about 10° to about 30°. The patent fails, however, to report the high speed formation defect termed herein the rippling effect, and does not teach the criticality of the velocity ratios as between the fibers and the forming surface in alleviating the detrimental rippling effect. Indeed, the present invention teaches that there are combinations of fiber stream velocities and forming surface velocities for which ducts aligned as recommended in Gotchel will produce unacceptable webs with pronounced ripples.

This invention relates to methods for forming a nonwoven fibrous web on a foraminous forming surface moving at a speed in excess of about 500 feet per minute (2.54 m/sec). The methods include dispersing the fibers uniformly in a gaseous medium to form a gaseous suspension of fibers. The gaseous suspension of fibers is conveyed in a stream to the moving forming surface onto which the fibers from the gaseous suspension are deposited to form a nonwoven fibrous web. The detrimental high-speed forming phenomenon termed the rippling effect is alleviated by controlling the critical relationship between the velocity of the fibers being deposited onto the moving forming surface, relative to the velocity of the latter.

According to the present invention, there is provided a method for forming a nonwoven fibrous web from fibers of a papermaking length generally less than inch (6.35 mm), wherein the fibers are distributed in a gaseous medium to form a gaseous suspension of fibers and are thereafter deposited from the gaseous suspension onto a moving foraminous forming surface to form the nonwoven fibrous web, characterised by the steps of
(a) moving the forming surface at a velocity Vₒ not less than 500 feet per minute (2.54 m/sec), and
(b) conveying the gaseous fiber suspension in a stream to the moving forming surface, the gaseous stream having a velocity component V, in the direction of motion of the forming surface and a velocity component V₂ normal to the forming surface, the magnitude of the difference between the forming surface velocity Vₒ and velocity component V, being less than 3 times the fiber velocity component V₂.

The forming surface onto which the fibers are deposited need not be planar, but could be curved, in which case it will have a tangential velocity Vₒ greater than 500 feet per minute (2.54 m/sec), the fiber velocity component V, being directed in the same direction as the motion of the curved forming surface.

When the velocities meet this ratio of 3:1 or less, the air-laid product is generally acceptable in terms of the ripple effect; outside this ratio the air-laid product generally is unacceptable as having excessive ripple characteristics.

In more complicated air/fiber flow patterns, wherein the gaseous stream containing the fibers has a further velocity component V₃ in the cross machine direction, the magnitude of the relative velocity component of the gaseous stream tangential to the forming surface, V' is equal to the square root of the quantity (Vₒ - V₁)² plus (V₃)². In this case also, the velocity V' should be less than about three (3) times the fiber velocity V₂.

Operation within the critical relationship between the fiber velocities relative to the forming surface velocity can be implemented in a variety of ways. For a given velocity Vₒ of the forming surface, the normal fiber velocity V₂ can be increased, for example by increasing the amount of suction pulling the gaseous stream through the moving surface. As a second example, the gaseous stream can be deflected to impinge upon the forming surface at an oblique angle, thereby increasing the velocity component Vl- of the gaseous stream in the direction of motion of the forming surface while maintaining velocity V₂ constant by increasing the amount of suction. In either approach the ratio of the velocity of the fibers relative to the velocity of the moving forming surface, compared to the component of the fiber velocities normal to the forming surface, can be varied to produce more acceptable pro₋ ducts having more uniform web characteristics.

The invention will now be described in more detail by way of non-limiting example, with reference to the accompanying drawings, in which:
FIGURES 1A and 1B illustrate air laid webs produced at velocity ratios (as hereinbefore mentioned) of 2.5:1 and 3.5:1, respectively;
FIGURES 2A and 2B are diagrams illustrating the ripple effect at velocity ratios of 1.3:1 and 4: 1, respectively;
FIGURE 3 is a graph illustrating ripple wavelength for velocity ratios of from 1 : 1 to 5:1; and
FIGURE 4 illustrates apparatus for use in practising this invention, with partial cutouts for clarity.

We have found that the high speed production of air laid webs is severely limited by a nonuniformity of web formation herein termed the ripple effect. This invention aims at alleviating the detrimental ripple effect by controlling certain critical relationships between the velocity of fibers in a gaseous stream being condensed on a moving foraminous forming surface, relative to the velocity of the moving surface.

Figures 2A and 2B illustrate two conditions of air laid web formation under two different velocity conditions as viewed relative to the surface 12. In Figure 2A, typical fiber paths, 10, illustrate fibers approaching a forming surface 12 at an overall relative velocity V (relative), relative to the surface 12. As shown, this overall relative velocity V (relative) is how an oncoming fiber would be viewed from a stationary point riding on the moving surface 12. The relative velocity, therefore, is the vector sum of the actual fiber velocity, here shown as V (actual) which has vector components V₂ normal to the forming surface and V, parallel to the forming surface 12. When viewed relative to the forming surface 12 moving at a velocity Vₒ, the velocity V, component is subtracted from Vₒ to obtain the fiber velocity V' relative to the surface 12. The magnitude of Vₒ - V, therefore represents the relative velocity of the oncoming fiber in a direction along the forming surface, and V₂ represents the velocity of the oncoming fiber in the direction normal to the forming surface. We have determined that a critical parameter in the formation of a web as illustrated in Figure 1A is the ratio of V' to the fiber velocity V₂ normal to the surface. We have found that in forming a nonwoven fibrous web substantially comprising fibers of a papermaking length generally less than inch (6.35 mm), this ratio must be maintained below about 3:1 to obtain acceptable product in terms of uniformity of the web, i.e. in terms of the inherent ripple effect.

Figure 2A further illustrates this ripple effect and our present belief of the reasons for the nonuniform web formation. Figure 2A illustrates a nonwoven web 14 formed of fibers deposited, as illustrated, along fiber paths 10. As the fibers are deposited on the forming surface 12, the fibers approach the surface at an oblique angle as viewed in a coordinate system moving with the forming surface. The ripple is believed to be primarily caused by a "shadowing" effect caused by the oblique approach of the fibers to the surface 12. This shadowing begins with the first fiber deposits, which occur randomly on the surface 12. These fiber deposits cause "shadows" directly downstream from their positions generally preventing oncoming fibers from falling in the areas of the shadows. Fiber continues to accumulate directly upstream from these initial deposits such as in thicker web portions 13 until the shadowing influence of a neighboring upstream deposit interferes. With further fiber deposition there is an apparent linking up of fiber deposits 13 in the cross machine direction to form the characteristic ripple effect. As is apparent from the Figure, this shadowing phenomenon produces the ripple effect with thicker web portions 13 alternating with thinner web portions 15. Further fiber deposition only increases the ripple characteristic of the web without changing the ripple wavelength. Except for some possible fiber bouncing or slipping during the initial deposition of fibers onto a surface, no fiber bouncing or slipping has been observed in the formation of webs below a velocity ratio of about 3:1. At ratios above about 3:1, fiber bouncing or slippage was observed to be a more significant forming phenomenon, with the resulting web exhibiting extremely nonuniform web characteristics.

Figures 2A and 2B illustrate the relation between the nonuniformity of web formation, i.e. the ripple effect, and the ratios between the fiber and forming surface velocities. In Figure 2A, V', the difference between velocity Vₒ of the moving surface 12 and velocity component V, of the fibers in the direction of motion of the surface, is about one and three tenths (1.3) times the velocity V₂ of the fibers normal to the moving surface, i.e. a velocity ratio- of 1.3. The resulting web, 14, is relatively uniform with closely spaced thicker web portions 13. In Figure 2B, the difference V' between velocity Vₒ of the moving surface 12_{B} and velocity component V, of the fibers in the direction of motion of the surface, is about four times that of velocity V₂ of the fibers normal to the moving surface 12g, (a velocity ratio of 4:1) and the-resulting web 14_{B} is much less uniform than the web 14 of Figure 2A, with a more pronounced ripple effect, i.e. with the thicker portions 13_{B} of the web more widely spaced and of greater relative basis weight than in the web 14 of 2A.

Figures 2A and 2B illustrate fiber velocities only having components V, in the direction of motion of the forming surface and V₂ normal to the forming surface. No fiber velocity components in the cross-machine direction, i.e. perpendicular both to velocity component V, and to velocity component V₂, have been illustrated since such velocity components are generally undesirable in the manufacture of air laid webs. In instances where such cross-machine velocity components do in fact exist, such velocity components V₃ may affect the web formation since those cross-machine velocity components will increase the relative velocity V' by the following formula, V' is equal to the square root of (Vₒ - V,)² + (V3)2, and thereby. affect the velocity ratio V':V₂. Such cross machine velocities V₃ may deleteriously affect the web, requiring corresponding adjustments to reduce V' or increase V₂ in those affected web areas.

Figures 1A and 1B are plan views of webs formed at velocity ratios of 2.5:1 and 3.5:1, respectively. As seen in Figure 1A, at the lower 2.5:1 ratio, the web produced is relatively uniform, exhibiting the ripple effect to a minor, but acceptable degree. Some variation in fiber deposit is evident, with recurring heavier deposits at, for example, 17A, 17B, 17C. As seen in Figure 1A, the distances between these uniformly recurring heavier deposits 17A, 17B, 17C can be measured and are termed the "wavelength" of the "ripples". As seen in Figure 1 B, web formed at a velocity ratio of 3.5:1 exhibits a ripple effect of far greater wavelength with thicker portions 19A, 19B, 19C, interspersed with thinner portions 19D and 19E. The web of Figure 1B is far less uniform in basis weight than the web of Figure 1A and is generally unacceptable.

Figure 3 is a graph illustrating experimental results of studies as to the ripple effect, for velocity ratios (V₀ ― V₁ : V₂) ranging from 1:1 to 5:1. These studies were conducted using softwood Kraft and included studies of other variables in the air laid forming process in order to verify the criticality of this velocity ratio parameter.

The tests verified that the ratio results as illustrated by Figure 3 are independent of the absolute speeds involved, from about 250 feet per minute (1.27 m/sec) up to a forming surface speed of about 2250 feet per minute (11.43 m/sec). It is believed that the ratio results are independent of speed at speeds lower than 250 feet per minute (1.27 m/sec) and greater than 2250 feet per minute (11.43 m/sec). Other tests verified that the ratio results as illustrated by Figure 3 are generally independent of the foraminous forming surface used for web formation at ratios of below 3:1. Most of the tests were conducted using a 59 (MD) x 42 (CD) brass forming wire, 0.0095 inch (MD) (0.241 mm) and 0.0115 inch (CD) (0.292 mm) in diameter. Other tests verifying these ratio results were conducted on wires: 40 (MD) x 32 (CD), bronze, 0.0112 inch (MD) (0.284 mm) x 0.0125 inch (CD) (0.317 mm); 78 (MD) x 64 (CD), bronze, 0.0067 inch (MD) (0.170 mm) x 0.00725 inch (CD) (0.0184 mm), 108 (MD) x 64 (CD) double-weave polyester 0.00866 inch (MD) (0.220 mm) x 0.00866 (CD), top, and 0.0118 (CD) (0.300 mm) bottom; and 84 (MD) x 32 (CD) two-layer polyester, 0.0157 inch (MD) (0.399 mm) x 0.0157 inch (CD) (0.399 mm). In the foregoing, the numbers preceding "(MD)" and "(CD)" refer to the number of mesh openings per inch (25.4 mm), considered in the direction of motion of the forming surface and transverse to this direction, respectively.

As shown in Figure 3, up to the critical velocity ratio of approximately 3: 1, the ripple wavelength, as defined above, increases to a minor degree with an increase in the velocity ratio. Air laid fibrous product produced under conditions of a velocity ratio of 3:1 or less, was generally considered to be acceptable in terms of uniformity of web density. Product produced at conditions of greater than a 3:1 velocity ratio was judged unacceptable in that the variances in web basis weight and thickness, the ripple effect, were too great. As seen in the graph of Figure 3, above the 3:1 ratio the variation in web characteristics becomes extremely disproportionate to a variation in velocity ratio, thereby establishing the criticality of the 3:1 limit.

Most of the studies establishing the criticality of the velocity ratio of 3:1 were conducted using softwood Kraft fibers which are relatively long cellulosic natural fibers. Use of fibers of other sizes would vary the ripple effect in terms of the wavelength but would not affect the criticality of the 3:1 ratio. For example, use of a shorter natural fiber such as a hardwood fiber, will cause less of the shadowing problem and will tend to shorten the wavelength in the web for a given velocity ratio.

Since lowering the velocity ratio will lower the ripple wavelength for a given length of fibers, the actual ratio at which the fibrous product is produced for commercial application can be varied to obtain a desired product. For example, it may be desired to produce fibrous product comprised substantially of softwood Kraft fibers at a velocity ratio of 2.5:1 for commercial purposes since that product would exhibit more uniform web characteristics than if produced at a 3:1 velocity ratio. Similarly, the fibrous product could be varied as to its composition, varying the fiber sizes to vary the ripple effect at a given velocity ratio. For example, a mixture of hardwood and softwood fibers might constitute commercially acceptable fibrous product at a higher velocity ratio than for a product produced primarily of softwood fibers.

As stated above, the wavelength of the ripple effect is independent of the overall basis weight of the deposited web. As the web is being deposited onto the forming surface, the spacing between the thicker portions of the web (the ripple wavelength) is established early during the deposition of the fibers, and further fiber deposition only increases the web thickness without affecting this ripple wavelength. For commercial purposes, a lower weight web, such as a tissue product, might be produced at a lower velocity ratio to shorten the ripple wavelength, obtaining a more satisfactory commercial product in terms of minimizing the effect of the thinner web portions 15. It is believed that this invention can be used to produce air laid webs at least in the range of from about 7 to about 75 pounds (3.17 to 34.01 kg) per 3000 square feet of web (278.7 sq. meters). The weight of fibers distributed over this area can be in the range 25 to 70 pounds (11.3 to 31.7 kg), for instance 30 to 45 pounds (13.6 to 20.4 kg).

The apparatus of Figure 4 illustrates an application of this invention to enable the production of acceptable air-laid web at a higher speed of production than previously possible.

In Figure 4, apparatus 18 comprises a conventional fiber distributor 20 positioned above a moving foraminous forming surface 22 moving from left to right in the drawing in the direction shown, with cellulosic fibers being impelled from the bottom 24 of the distributor 20 to form an air suspension of fibers directed toward the forming surface 22. A suction box 26 is positioned below the forming surface 22, offset somewhat in the downstream direction relative to the distributor 18, the suction box 26 in use creating a moving air stream downwardly through the forming surface 22 and out via an exhaust pipe 28 to a fan (not shown).

The air stream fibers flow from the bottom 24 of the distributor box to the portion of the moving surface 22 above the suction box 26 where the fibers are deposited in the form of an air laid web 29. In this stream of fibers, the individual fibers are brought onto the moving surface 22 at an oblique angle by means of both the action of the offset position of the suction box 26 as well as by air turning foils 30. The turning foils 30 are positioned adjacent the upstream end of the distributor 20 and generally serve to introduce a horizontal air stream into the stream of fibers flowing from the distributor 20 to the forming web 22. Sealing roll 32 is positioned along the downstream end of distributor 20 substantially to seal the space between the distributor 20 and the forming surface 22. Side seals, not shown, seal the sides of the apparatus. These seals reduce air loss and minimize air turbulence within the apparatus.

The horizontal air stream introduced by the turning foils 30 coacts with the offset suction box 26 to impart a horizontal component of velocity to the fibers within the airstream. The dashed lines L in Fig. 4 indicate typical probable paths of fibers and illustrate that the fibers approach the moving surface 22 at an oblique angle having a velocity component in the direction of movement of the moving wire 22, thereby enabling the production of an acceptable air laid web at a higher speed of the forming surface 22 in accordance with this invention.

## Claims

1. A method for forming a nonwoven fibrous web from fibers of a papermaking length generally less than inch (6.35 mm), wherein the fibers are distributed in a gaseous medium to form a gaseous suspension of fibers, and are thereafter deposited from the gaseous suspension onto a moving foraminous forming surface to form the nonwoven fibrous web, characterised by
(a) moving the forming surface at a velocity Vₒ not less than 500 feet per minute (2.54 m/sec), and
(b) conveying the gaseous fiber suspension in a stream to the moving forming surface, the gaseous stream having a velocity component V, in the direction of motion of the forming surface and a velocity .component V₂ normal to the forming surface, the magnitude of the difference between the forming surface velocity Vₒ and velocity component V, being less than 3 times the fiber velocity component V₂.

2. The method according to claim 1, characterised by the magnitude of the relative difference between velocity Vₒ and velocity component V, being less than 2.5 times the fiber velocity component V₂.

3. The method according to claim 1 or claim 2, characterised in that the fibers are laid on a forming surface which is a screen comprised of 40 brass wires, each 0.0125 inch (0.317 mm) transverse to the direction of movement of the screen, and 60 brass wires, each 0.0112 inch (0.284 mm) in the said direction.

4. The method according to claim 1, 2 or 3, characterised in that the fibers are deposited onto the forming surface to form a nonwoven fibrous web having a basis weight in the range of from 7 to 75 pounds (3.17 to 34.01 kg) per three thousand square feet (287.7 sq. m) of web.

5. The method according to claim 4, characterised in that the fibers are deposited to form a nonwoven fibrous web having a basis weight in the range of 25 to 70 pounds (11.3 to 31.7 kg) over the said web area.

6. The method according to claim 4, characterised in that the fibers are deposited to form a nonwoven fibrous web having a basis weight in the range of 30 to 45 pounds (13.6 to 20.4 kg) over .the said web area.

7. The method according to any of claims 1 to 6, characterised by the relative difference between velocity Vₒ and velocity component V, being less than twice the normal fiber velocity component V₂.

8. The method according to any preceding claim, characterised by the gaseous stream having a further velocity component V₃ in a direction perpendicular both to velocity component V, and to velocity component V₂; the magnitude of the square root of (V₀ ― V₁)² + (V₃)², being less than 3 times the normal fiber velocity component V₂.

9. The method according to any of the preceding claims, characterised in that the fibers are deposited on a curved forming surface which has a tangential velocity component Vₒ greater than 500 feet per minute (2.54 m/sec), the fiber velocity component V₁ being directed in the same direction as the motion of the curved forming surface.

## Revendications

1. Procédé pour former une nappe fibreuse non tissée à partir de fibres d'une longuer pour papeterie, généralement inférieure à 6,35 mm ( inch) dans lequel les fibres sont distribuées dans un milieu gazeux pour former une suspension gazeuse de fibres, et sont ensuite déposées de la suspension gazeuse sur une surface poreuse de mise en forme en mouvement pour former la nappe fibreuse non tissée, caractérisé en ce qu'il consiste:
(a) à déplacer la surface de mise en forme à une vitesse Vₒ non inférieure à 2,54 m/s (500 feet par minute), et
(b) à transporter la suspension gazeuse de fibres en un courant vers la surface de mise en forme en mouvement, le courant gazeux ayant une composante de vitesse V, dans la direction du mouvement de la surface de mise en forme et une composante de vitesse V₂ normale à la surface de mise en forme, l'amplitude de la différence entre la vitesse Vₒ de la surface de mise en forme, et la composante de vitesse V, étant inférieure à trois fois la composante V₂ de vitesse des fibres.

2. Procédé selon la revendication 1, caractérisé en ce que l'amplitude de la différence relative entre la vitesse Vₒ et la composante de vitesse V, est inférieure à 2,5 fois la composante V₂ de vitesse des fibres.

3. Procédé selon la revendication 1 ou la revendication 2, caractérisé en ce que les fibres sont appliquées sur une surface de mise en forme qui est une toile constituée de 40 fils de laiton, chacun de 0,317 mm (0,0125 inch), transversaux à la direction du mouvement de la toile, et 60 fils de laiton, chacun de 0,284 mm (0,0112 inch), dans ladite direction.

4. Procédé selon la revendication 1, 2 ou 3, caractérisé en ce que les fibres sont déposées sur la surface de mise en forme pour former une nappe fibreuse non tissée ayant une force dans la plage de 3,17 à 34,01 kg (7 à 75 pounds) par 278,7 m² (3000 square feet) de nappe.

5. Procédé selon la revendication 4, caractérisé en ce que les fibres sont déposées pour former une nappe fibreuse non tissée ayant une force dans la plage de 11,3 à 31,7 kg (25 à 70 pounds) sur ladite surface de la nappe.

6. Procédé selon la revendication 4, caractérisé en ce que les fibres sont déposées pour former une nappe fibreuse non tissée ayant une force de 13,6 à 20,4 kg (30 à 45 pounds) sur ladite surface de la nappe.

7. Procédé selon l'une quelconque des revendications 1 à 6, caractérisé en ce que la différence relative entre la vitesse Vₒ et la composante de vitesse V₁ est inférieure au double de la composante de vitesse normale V₂ des fibres.

8. Procédé selon l'une quelconque des revendications précédentes, caractérisé en ce que le courant gazeux possède une autre composante de vitesse V₃ dans une direction perpendiculaire à la fois à la composante de vitesse V, et à la composante de vitesse V₂; l'amplitude de la racine carrée de (V₀ ― V₁)² + (V₃)² étant inférieure à trois fois la composante de vitesse normale V₂ des fibres.

9. Procédé selon l'une quelconque des revendications précédentes, caractérisé en ce que les fibres sont déposées sur une surface incurvée de mise en forme qui possède une composante de vitesse tangentielle Vₒ supérieure à 2,54 m/s (500 feet par minute), la composante de vitesse V, des fibres étant dirigée dans la même direction que le mouvement de la surface incurvée de mise en forme.

## Patentansprüche

1. Verfahren zur Bildung einer Faservliesbahn aus Fasern einer für die Papiererzeugung geeigneten Länge von allgemein weniger als 6,35 mm, wobei die Fasern in einem gasförmigen Medium verteilt werden unter Bildung einer gasförmigen Fasersuspension und anschließend aus der gasförmigen Suspension auf eine bewegte, Perforationen aufweisende Formoberfläche abgeschieden werden unter Bildung der Faservliesbahn,. gekennzeichnet durch
(a) Bewegen der Formoberfläche mit einer Geschwindigkeit Vₒ von nicht weniger als 2,54 m/s; und
(b) Fördern der gasförmigen Fasersuspension in einem Strom zu der bewegten Formoberfläche,. wobei der gasförmige Strom eine Geschwindigkeitskomponente V₁ in Bewegungsrichtung der Formoberfläche und eine Geschwindigkeitskomponente V₂ senkrecht zur Formoberfläche hat und die Differenz zwischen der Geschwindigket Vₒ der Formoberfläche und der Geschwindigkeitskomponente V, kleiner als die 3fache Fasergeschwindigkeitskomponente V₂ ist.

2. Verfahren nach Anspruch 1, dadurch gekennzeichnet, daß die relative Differenz zwischen der Geschwindigkeit Vₒ und der Geschwindigkeitskomponente V, kleiner als die 2,5fache Fasergeschwindigkeitskomponente V₂ ist.

3. Verfahren nach Anspruch 1 oder 2, dadurch gekennzeichnet, daß die Fasern auf eine Formoberfläche gelegt werden, die ein Sieb aus 40 Messingdrähten von jeweils 0,317 mm, die quer zur Bewegungsrichtung des Siebs verlaufen, und 60 Messingdrähten von jeweils 0,284 mm, die in der gennanten Richtung verlaufen, ist.

4. Verfahren nach Anspruch 1, 2 oder 3, dadurch gekennzeichnet, daß die Fasern auf die Formoberfläche abgeschieden werden unter Bildung einer Faservliesbahn mit einer Masse von 3,17-34,01 kg je 278,7 m² der Bahn.

5. Verfahren nach Anspruch 4, dadurch gekennzeichnet, daß die Fasern abgeschieden werden unter Bildung einer Faservliesbahn mit einer Masse von 11,3-31,7 kg über die genannte Bahnfläche.

6. Verfahren nach Anspruch 4, dadurch gekennzeichnet, daß die Fasern abgeschieden werden unter Bildung einer Faservliesbahn mit einer Masse von 13,6-20,4 kg über die genannte Bahnfläche.

7. Verfahren nach einem der Ansprüche 1-6, dadurch gekennzeichnet, daß die relative Differenz zwischen der Geschwindigkeit Vₒ und der Geschwindigkeitskomponente V, kleiner als die 2fache senkrechte Fasergeschwindigkeitskomponente V₂ ist.

8. Verfahren nach einem der vorhergehenden Ansprüche, dadurch gekennzeichnet, daß der Gasstrom eine weitere Geschwindigkeitskomponente V₃ in einer Richtung, die sowohl zur Geschwindigkeitskomponente V₁ als auch zur Geschwindigkeitskomponente V₂ senkrecht verläuft, hat; wobei die Größe der Quadratwurzel aus (V₀ ― V₁)² + (V₃)²kleiner als die 3fache senkrechte Fasergeschwindigkeitskomponenete V₂ ist.

9. Verfahren nach einem der vorhergehenden Ansprüche, dadurch gekennzeichnet, daß die Fasern auf eine gewölbte Formoberfläche abgeschieden werden ,die eine tangentiale Geschwindigkeitskomponente Vₒ von mehr als 2,54 m/s hat, wobei die Fasergeschwindigkeitskomponente V₁ in dieselbe Richtung wie die Bewegung der gewölbten Formoberfläche gerichtet ist.
